

## UNITED STATES PATENT OFFICE.

CARL C. KESLER, OF PITTSBURGH, PENNSYLVANIA, ASSIGNOR TO PINE INSTITUTE OF AMERICA, INCORPORATED, OF JACKSONVILLE, FLORIDA, A CORPORATION OF DELAWARE.

## PROCESS OF MAKING ROSIN SOAP.

No Drawing.

Application filed July 30, 1925. Serial No. 47,123.

My invention relates to the treatment of rosin and the production of rosin soap.

Rosin is a substance of wide industrial utility, but, because of certain characteristics, it serves imperfectly some purposes for which it is used. In soap-making, for example, rosin is a useful substance. Added to and forming a mixture with the fatty-acid compounds of which soap essentially 10 consists, a commercial soap is produced which, as compared with a soap composed of fatty-acid compounds alone, is relatively inexpensive, more freely productive of lather, and of greater cleansing power. 15 The disadvantages incident to the use of rosin as an ingredient of soap are that cakes of soap which contain it are liable in time, particularly when exposed to humid air, to become moist and sticky. They also tend 20 to grow discolored. This tendency to become moist and sticky is such that hitherto it has not been possible to produce in satisfactory condition for the market rosin-containing soap in the form of soap chips. 25 And such a commodity is a recognized desideratum.

I have discovered, and from this discovery my invention proceeds, that by preliminary treatment of the rosin of commerce, resulting in a certain chemical change in its substance, and by an ensuing separation of constituents, substances may be obtained which are serviceable in the industrial arts, in fuller degree than rosin has been known to 35 be serviceable. In soap-making for instance, the rosin derivative of my invention, when mixed with the fatty-acid compounds from which soap is prepared, affords a commercial soap having the known good qualities of 40 rosin soap and free of the undesirable qualities which rosin soap as hitherto produced, has possessed. And, specifically, soap chips made from soap containing my rosin derivative are stable, and become a satisfactory 45 article of commerce, and fill a recognized want.

Abietic acid is a desirable substance, being useful for various industrial purposes, and in the practice of my invention I am able 50 to produce abietic acid free of impurities and this in economical manner.

Again in varnish-making, the treatment to which I subject rosin affords me resene, freed from abietic acid compounds, and

chemically pure or substantially so. The so 55 liberated resene, being a neutral gum having enhanced drying properties, serves as a valuable constituent of varnishes.

In the practice of my invention, and beginning with the rosin of commerce, I first, 60 by the known means of acid treatment or heat, isomerize the material. Specifically, by heating the rosin to a temperature of 300° C. and maintaining it at that temperature, isomerization may be effected. Or, again, 65 if the rosin be melted, and if while it remains in liquid condition a slow current of hydrochloric acid gas be caused to pass through it, isomerization will be effected. If while such acid treatment is in progress 70 stirring be resorted to, or other means for effecting more intimate contact of the substances so brought into association, isomerization may be effected in about fifteen 75 minutes.

Having effected isomerization of the rosin, I dissolve it in a suitable solvent, such as ethyl alcohol, methyl alcohol, or other alcohol and to the solvent either before or after solution I add sodium hydroxide, or other 80 alkali, in the amount of one fourth of the equivalent weight of the rosin under treatment. A convenient degree of concentration of the sodium hydroxide employed would be a forty per cent, aqueous solution, 85 but it will be understood that the degree of concentration does not enter into the essence of the invention, and the degree of concentration may in fact vary indefinitely. The sodium hydroxide may be added to the solution in any suitable precipitating tank, fitted with steam coils for heating and with agitators for stirring. After the addition the material is allowed to stand for a short time, until the reaction and precipitation are 90 complete. The material being stirred, is mobile enough to be pumped.

The material then is carried to a filter press, where the precipitate is separated. The filtrate which passes on carries with it 100 in solution the resene, and this substance may now be recovered free of abietic acid compounds.

The precipitate which remains in the filter press consists of an alkali metal (sodium) 105 acid salt of abietic acid. This added to the fatty-acid compounds of which soap is essentially prepared, affords a commercial soap

of the excellence indicated, and a soap which may be prepared and marketed in the form of chips, which are serviceable and satisfactory.

5 The precipitate remaining in the filter press may be used as it is, or it may be purified of all trace of resene by washing it with more of the solvent. It may by pressure be freed sufficiently of solvent, or, if more 10 complete removal of the solvent be desired, the cake from the filter press may be heated, and the last trace of solvent may be drawn off, preferably under vacuum. The resene-containing solvent so ultimately separated 15 from the precipitate, may of course be returned to the main body of solvent, and its burden of resene in such manner saved.

The procedure here outlined may advantageously be carried out in closed system, as 20 the practitioner of the art will well understand.

Having by the procedure described obtained in pure condition an alkali metal acid salt of abietic acid, it remains only to treat 25 the salt with a mineral acid, hydrochloric acid, for example, in order to obtain abietic acid of corresponding purity.

I find that in the practice of my invention

upon the rosin of commerce a yield of pure acid amounting to seventy-five to eighty per cent by weight of the quantity of rosin treated may be recovered. 80

In the ensuing claims I use the term alkali metal, and I use it in its wider significance, to include ammonium. 85

I claim as my invention:

1. The method herein described of producing rosin soap which consists in converting the major part of the acid component of a quantity of rosin into alkali acid salt, 40 removing from such salt the resene component of the rosin, and using the remaining salt as an ingredient in the soap-making operation.

2. The method herein described of producing rosin soap which consists in isomerizing a quantity of rosin, bringing the so treated substance into solution, precipitating from such solution an alkali metal acid salt of abietic acid, separating the precipitate, 45 and introducing the separated precipitate as an ingredient in the soap-making operation.

In testimony whereof I have hereunto set my hand.

CARL C. KESLER.